

## UNITED STATES PATENT OFFICE.

ALBERT F. FRENCH, DECEASED, LATE OF DETROIT, MICHIGAN; BY MARY A. FRENCH, ADMINISTRATRIX, OF DETROIT, MICHIGAN.

## FILLER COMPOSITION.

No Drawing.

Application filed July 26, 1922. Serial No. 577,745.

To all whom it may concern:

Be it known that ALBERT F. FRENCH, deceased, a citizen of the United States of America, resident of Detroit, in the county 5 of Wayne and State of Michigan, has invented certain new and useful Improvements in Filler Compositions, of which the following is a specification.

This invention relates to a filling 10 pound, somewhat along the lines suggested in my Patent No. 1,352,741, granted Sept. 14, 1920, disclosing a filler composition that may be placed in cracks, scratches and scarred surfaces and afterwards varnished 15 or painted over to render the demarcations invisible. The present composition may be in liquid form and applied with a brush or it may be in the form of putty, especially for filling large cracks. In either form it will 20 not materially contract and will permit of an injured surface being expeditiously repaired or finished, in contradistinction to treatments requiring hours and sometimes 25 days to complete.

My composition consists of the following ingredients for compounding one gallon of the liquid filler:—

|                            |        |
|----------------------------|--------|
| Graphite (dry powder)----- | 2 lbs. |
| Fuller's earth-----        | 8 "    |
| Gum thus-----              | 1 "    |
| Turpentine.                |        |

To the gum thus is added enough turpentine to cut the gum and at the same time make one gallon of liquid filler which may 35 be applied to a surface with a brush. Less turpentine is added to the ingredients when only a paste or putty form is required, and should the filler putty be too light or thin it may be thickened with white lead.

Should the liquid form of filler be too 40 thick it may be thinned out by adding more turpentine.

In practice, a large crack is filled with the putty or paste form of the composition and 45 after setting for about a half hour or less it is gone over with the liquid form of the composition. The liquid form dries rapidly and then paint or varnish may be applied.

In the composition the gum thus serves as 50 a binder that will not contract; the fuller's

earth as a body for the composition and the graphite to provide a smooth finish or polish to a surface.

This composition, particularly in its liquid form, may be advantageously used in 55 the automobile industry for finishing automobile bodies. At present an automobile body, in its natural condition is provided with what is commonly known as "a sand oil surface," that is, it is coated with a liquid 60 containing oil or varnish. Then the body is placed in an oven to dry and then receives another surface of the same liquid, but the first applied coat is sand papered prior to the second coat being applied, and then the 65 body is returned to the oven to again be dried. This operation may be continued until the body has a desired surface and such operations are slow and tedious because considerable time is required in an oven for 70 drying, and the surfacing liquid retards sanding off the surface due to the oil and varnish in the surfacing liquid. Besides, from a commercial standpoint considerable 75 labor is involved and the maintenance of an oven expensive.

This composition, when used as a surfacer, dries in approximately a half hour without the aid of heat; contains no oil or varnish, saves sand paper and time incident to finishing off the first coated surface to receive the second coat, and materially increases production in any factory where vehicle bodies or other articles of manufacture are provided with highly finished surfaces. 85

From the foregoing it will be noted that this composition may be considered as a sand surfacer and considerable importance is attached to the gum thus as an essential element, which obviates the necessity of 90 using any oil or varnish.

What I claim is:—

1. A filler composition consisting of graphite, two pounds; fuller's earth, eight pounds; gum thus, one pound; and sufficient turpentine to cut the gum thus and make one gallon of the composition. 95

2. A filler composition comprising gum thus as an adhesive and binding material, turpentine as a solvent for the gum, 100

fuller's earth as a body, graphite as a smooth surface material, and in which composition fuller's earth amounts to over ninety per cent of the whole.

5 3. A filler composition comprising two parts graphite, eight parts fuller's earth, gum thus, and a volatile solvent for the gum in such quantities as to cause the gum

to serve as a binder for the graphite and earth.

MARY A FRENCH,  
*Administratrix of the Estate of Albert F.*  
*French, Deceased.*

Witnesses:

KARL H. BUTLER,  
G. E. McGANN.